

Sept. 11, 1928.

1,684,006.

**Q. BENT ET AL**  
**TREATMENT OF ORES**  
Filed Oct. 4, 1920



Inventors  
Quincy Bent,  
Edwin Barnhart,  
and  
Frederick W. Wood.  
By their Attorney

Clarence Kerr

Patented Sept. 11, 1928.

## UNITED STATES PATENT OFFICE.

QUINCY BENT, OF BETHLEHEM, PENNSYLVANIA; EDWIN BARNHART, OF SPARROWS POINT, MARYLAND; AND FREDERICK W. WOOD, OF PHILADELPHIA, PENNSYLVANIA, ASSIGNORS TO BETHLEHEM STEEL COMPANY, OF BETHLEHEM, PENNSYLVANIA, A CORPORATION OF PENNSYLVANIA.

## TREATMENT OF ORES.

Application filed October 4, 1920. Serial No. 414,705.

Fig. 1 shows an elevation of apparatus suitable for employment in carrying out our invention; Fig. 2 is a partial longitudinal section thereof; and Figs. 3 and 4 are sections on lines III—III and IV—IV, respectively, of Fig. 1.

Our invention relates to the treatment of ores, particularly those forms of ores which, in their natural state, occur in a finely divided condition, and, because of their liability to pack when wet, or blow out with the blast when dry, require treatment preparatory to sintering or other reduction in a furnace. We have found that our invention is particularly useful with ores, such as Mayari iron ore, which, because of its clay-like consistency when wet, prevents the passage of air or gas uniformly through the mass, and thereby renders sintering or other treatment difficult. By the employment of our invention, however, the ore is brought into such condition that it may be readily sintered or otherwise treated.

In the drawings we have shown apparatus of a character which may be suitably employed in carrying out our invention, and which consists in a rotary cylinder, preferably set at a slight angle to the horizontal, so that, as the material is picked up and let fall by lifting blades 2 with each revolution of the cylinder, it will be advanced toward the discharge end thereof. At the intake end 3 is a chute 4, through which the material is admitted into the cylinder, while the discharge end 5 is equipped with a screen 6, through which the smaller sizes of material will escape and thus be separated from the larger sizes. The discharge end 5 may be open, as shown, to permit the discharge of the larger agglomerations of the material. Beneath the screen 6 and open end 5 of the cylinder are arranged the pockets 7 and 8 for the reception, respectively, of the smaller and larger agglomerations of material, and from which the material is carried away by the conveyer belts 9 and 10. The cylinder is heated at its discharge end by a gas burner 11, or by any other suitable means.

As a typical example of carrying out our invention, we will describe its application to the treatment of Mayari ore from Cuba in

the apparatus just described. It is well known that the free moisture content of Mayari ore mentioned is much higher than required to produce the same physical consistency with other ores different in character.

The ore, in a form which normally contains from 25 to 30 per cent of free moisture, is introduced into the agglomerating zone A of the cylinder through the chute 4, and at the same time a charge of coke in pulverized form is fed in with the ore, the coke charge being preferably about 5 per cent of the amount of the ore. As the interior of the cylinder at its intake end 3, which is remote from the burner 11, is cold, the ore will adhere to it between the lifting blades 1, which serve to pick up the material and assist in agglomerating it. As the cylinder revolves, the material drops off in large chunks, which are beaten and picked up again and again by the blades 1 as the cylinder revolves, and which at the same time pick up additional globules of the material, which forms into balls and pellets. The balling action also assists in bringing a portion of the moisture of the material to the surface so that it is readily carried off by the heated air when the drying zone is reached. Because of the downward inclination of the cylinder toward its discharge end, the material is advanced toward that end with each revolution of the cylinder. The balling action is assisted in the drying zone B by the blades 2, which serve to roll the material and shape it in the form of balls or spheres. The material is preferably subjected as it approaches the discharge end to a comparatively low heat from the burner 11, and the moisture released thereby is carried off with the air by means of a fan 12, which is arranged at the intake end of the cylinder. We have found that where the material as it is introduced into the cylinder contains a free moisture content of from 25 to 30 per cent, that approximately from one-third to one-half of the moisture is eliminated as it passes through the cylinder.

The feed end of the rotary kiln should be relatively cold, it being a characteristic of wet plastic material, that it adheres more readily to a cold than to a warmed surface.

The temperature at the discharge end of the kiln should be kept to a moderate degree, so that only a portion of the total moisture may be removed. The amount of residual moisture to be left in the balls or pellets will somewhat depend on the nature and physical characteristics of the material under treatment. If insufficient moisture be removed, the balls tend to adhere one to another and 10 form sticky agglomerates of substantial size. If, on the other hand, a higher degree of heat be applied, so as to almost reduce the material to dryness, the cohesive and plastic character of the balls is destroyed in such 15 a manner that they may disintegrate to a more or less pulverulent condition.

The agglomerating and drying process is continued until the larger globules roll out at the discharge end 5 of the cylinder and 20 the finer globules sift through the screen 6 at such end, thus effecting an automatic sorting of the material.

An important feature of our invention is the fact that, the partial removal of 25 moisture at low temperatures does not cause any substantial shrinkage of the masses, so that the material composing the balls leaves the rotating cylinder in a porous condition, eminently suitable for subsequent furnace 30 treatment.

The material, when agglomerated into the form of balls or pellets by the process just described, is sufficiently hard to stand ordinary handling. Even when the balls are 35 of considerable size the material offers little resistance to the uniform passage of air or gas therethrough, and is therefore in condition for treatment by any of the well-known sintering or roasting processes. The 40 crushed fuel, which is added at the beginning of the balling or agglomerating process, is gathered up and embedded in the balls during their formation, and thereby insures a uniform and intimate mixture between the 45 ore and fuel, which is highly desirable in the subsequent reducing operations. The use of an additional agent, as for example carbonaceous material, though a convenience to certain further operations, is not, however, essential to the process.

The terms and expressions which we have employed are used as terms of description and not of limitation, and we have no intention, in the use of such terms and expressions, of excluding any equivalents of the features described, but recognize that various modifications are possible within the scope of the invention claimed.

What we claim is:

60 1. A process for rendering wet ores of plastic character suitable for a subsequent furnacing operation which consists in, feeding the ore into the cool end of an internally and longitudinally ribbed rotary kiln, 65 whereby the plastic ore mass may be divided

into a plurality of integral masses disposed longitudinally of the kiln, said kiln having its axis inclined to the horizontal and being rotated so as to carry the masses to a point at which they may become gravimetrically 70 detached and fall downwardly and forwardly in the kiln, causing said detached masses to be individually carried upward and dropped forwardly in the kiln by the continued rotation of the latter, whereby the 75 ore may be formed into masses of the size desired and submitting said masses during their downward tumbling passage through the kiln to a moderate degree of heat so as to effect a partial removal of their contained moisture.

2. A process for rendering wet ores of plastic character suitable for a subsequent furnacing operation which consists in, feeding the ore together with carbonaceous material into the cool end of an internally and longitudinally ribbed rotary kiln, whereby the plastic ore may be divided into a plurality of integral masses disposed longitudinally of the kiln, the kiln having its axis inclined to the horizontal and being rotated so as to carry the masses to a point at which they may become gravimetrically 80 detached and fall downwardly and forwardly in the kiln, causing said detached masses to be 85 individually carried upwardly and dropped forwardly in the kiln by the continued rotation of the latter, whereby the ore may be formed into masses of the size desired and submitting said masses during their downward tumbling passage through the kiln to a moderate degree of heat so as to effect a partial removal of their contained moisture.

3. A process for rendering wet ores of plastic character suitable for a subsequent furnacing operation, which consists in, adding to the ore material susceptible of reacting in a subsequent furnace operation with certain components of the ore, feeding the 105 mixture into the cool end of an internally and longitudinally ribbed rotary kiln, whereby the plastic ore may be divided into a plurality of integral masses disposed longitudinally of the kiln, the kiln having 110 its axis inclined to the horizontal and being rotated so as to carry the masses to a point at which they may become gravimetrically 115 detached and fall downwardly and forwardly in the kiln, causing said detached masses to be 120 individually carried upwardly and dropped forwardly in the kiln by the continued rotation of the latter, whereby the ore may be formed into mases of the size desired, and submitting said masses during their downward tumbling passage through the kiln to a moderate degree of heat so as to effect the partial removal of their contained moisture.

4. A process for converting a plastic ad- 130

hesive conglomerate into a plurality of non-adhesive units suitable for subsequent furnace treatment, which consists in, feeding the material into the charging end of an inclined rotary kiln internally and longitudinally ribbed so as to sub-divide the conglomerate into a plurality of integral masses, raising, inverting and dropping said masses in repeating sequence by the continued rotation of the kiln, the inclination of the latter being such as to cause the masses to move gradually forward into a zone of moderate heat disposed towards its discharge end, said heat being of a degree sufficient to effect a partial removal of moisture from the separate integral masses, "balled" by their tumbling movement into the zone of heat aforesaid.

5. A process for forming an impervious conglomerate into a plurality of substantially porous units suitable for subsequent furnace treatment, which consists in, feeding the conglomerate and carbonaceous material into the charging end of an inclined rotary kiln internally and longitudinally ribbed so as to sub-divide the conglomerate into a plurality of integral masses, raising, inverting and dropping said masses in repeating sequence by the continued rotation 20 of the kiln, the inclination of the latter being such as to cause the masses to move gradually into a zone of moderate heat disposed towards its discharge end, and limiting said temperature so that the separate 25 integral masses "balled" by their tumbling movement into the zone of heat, may be

rendered porous by the partial evaporation of their contained moisture.

6. A process for rendering wet ores of plastic character suitable for subsequent 40 furnace treatment, which consists in, forming integral slabs of the ore on the internal periphery of an inclined rotating kiln, having a zone of moderate heat disposed at its discharge end, causing said slabs to be repeatedly tumbled and carried forwardly into the zone of heat by the rotation of the kiln, whereby the slabs may be formed into substantially ball-like members, limiting the 45 temperature of said zone so as to effect only 50 a partial evaporation of the moisture contained in the members, and finally grading the members by a process of screening.

7. A process for rendering wet ores of plastic character suitable for subsequent 55 furnace treatment, which consists in, forming integral slabs of the ore with carbonaceous material added thereto on the internal periphery of an inclined rotary kiln, the kiln being provided at its discharge end 60 with a zone of moderate heat, causing said slabs to be repeatedly tumbled and carried into the zone of heat by the rotation of the kiln, whereby the slabs may be formed into substantially ball-like members, limiting the 65 temperature of said zone so as to effect only a partial evaporation of the moisture contained in the members, and finally grading the members by a process of screening.

QUINCY BENT.

EDWIN BARNHART.

FREDERICK W. WOOD.